

## UNITED STATES PATENT OFFICE

2,165,392

TREATMENT OF TEXTILE MATERIAL AND  
PRODUCT THEREOF

Leon Lillienfeld, Vienna, Austria

No Drawing. Application June 22, 1932, Serial  
No. 618,804. Renewed March 15, 1938. In  
Great Britain July 4, 1931

19 Claims. (Cl. 91—68)

The present invention relates to a process of treating textile material (whether in the form of woven fabrics or spun goods such as yarn) by coating, impregnating, filling, dressing, weighting, sizing, printing or the like by means of cellulose or of cellulose derivatives or of cellulose compounds. It is based on the discovery that the textile materials attain excellent properties when the cellulose or its derivatives or compounds are deposited on, or in the fibers of the textile material from a lather into which a solution of cellulose or of a cellulose derivative or a cellulose compound has been transformed before being applied to the textile material.

15 In my U. S. Patents No. 1,829,904 and No. 1,829,905, I have disclosed a process of treating fibrous material by applying to it, by a dressing, sizing, printing, weighting or like operation, an emulsion of air or gas bubbles in a viscous solution of a cellulosic material (such as viscose), from which cellulose can be regenerated or precipitated, in which solution a gas has been dissolved or otherwise dispersed, i. e. emulsified, (for example by injection, blowing, beating, or 20 by solution of the gas in the liquid under pressure or by dissolving a gas-liberating salt such as sodium carbonate, in such solution) and thereafter treating the material to regenerate or precipitate the cellulose, so as to produce a composite material comprising fibrous material associated with a dressing or sizing of regenerated cellulose containing hollow spaces or bubbles dispersed throughout it or throughout a part of it. A convenient way of obtaining the solution from which cellulose may be regenerated or precipitated consists for example in injecting air or another gas into a viscose so as to produce an "emulsion" of gas bubbles in the viscose. There 25 may be added to the viscose or cellulose solution various other substances, for instance softening agents such as glycerine, soap, Turkey-red oil, glucose, castor oil or paraffin oil.

I have now found that the application of the solution of paste of cellulosic material, in the 30 form of a lather, (instead of emulsion) in accordance with the process of the present case produces a surprising difference in the properties of the treated fibrous material and gives a far greater economy of the process, these results being achieved by treating the solution from which cellulose may be regenerated or precipitated, before applying the same to the textile material, in such a manner as to convert it into a lather.

The advantageous properties of the coatings, 35 coverings, dressings, fillings, sizings, printings,

and finishings made according to the present invention are, for example, their attractive appearance, their pleasant, warm and rich feel to the touch, their great voluminosity, their downy character and very low specific gravity. In all 5 these respects the final products of the present invention surpass the products obtainable according to the known processes (as in my said prior patents) of incorporating with textile materials cellulose or cellulose compounds in the 10 form of coatings, dressings, sizings, fillings, weighting materials or printing layers which contain hollow spaces produced by emulsions of air or any other gas in solutions or pastes of cellulose or cellulose conversion products or cellulose 15 compounds. The characteristic feature of the present invention—the lathery condition of the solutions or pastes—being absent in the emulsions prepared according to the processes known heretofore, the voluminosity, specific gravity, softness and feel of the final products made according to the known processes are distinctly inferior to the voluminosity, softness, feel and specific gravity of the final products of the present invention. The capability of the invention of imparting the greatest possible volume to its initial materials (that is to say, to the solutions or pastes of cellulose or of its conversion products or derivatives) and, what is more important, to 25 its final products, appears to be unrivaled in its 30 domain of application.

To show that the apparent specific gravity of the cellulose or of the cellulose derivative deposited on, or in, the textile fibre in the present invention is almost incredibly lower than the 35 apparent specific gravity of the cellulose deposited on, or in, the fibre in the processes in which emulsions (as in Patent 1,829,905) of a gas in viscose or cellulose solutions are used, I adduce the following example: Whilst the apparent specific gravity of cellulose regenerated from viscose in, or on, the fibre is about 1.5 to 1.6, and whilst the apparent specific gravity of the cellulose deposited in, or on, the fibre from an emulsion of a gas in viscose (for example according to the process described in my U. S. Patent 1,829,905) is, at the outside, 1.2 to 1.3, according to the present invention it is possible to reduce the apparent specific gravity of the cellulose regenerated from viscose far below 1.2 and 40 even down to 0.5 or even down to 0.1 to 0.2. This 45 fact alone proves that, from the viewpoint of economy and, what is more important, with regard to lightness, softness and downy character of the dressings and sizings, the advantages of 50 55

the present process over all known processes in which cellulosic bodies by themselves or associated with hollow spaces are deposited within textile materials, may be looked upon as very great.

5 A striking feature of the present invention is the fact that, in spite of its extremely spongy or lathery condition, the cellulose or the cellulose compound or cellulose derivative associated with the textile material according to the present invention is so intimately amalgamated with the textile fibre that the fastness towards rubbing, or bending or laundering of the final products is even then highly remarkable even when unusually large amounts of mineral fillers (for example talc or china clay) are incorporated with the lather or the solution or paste to be transformed into lather.

10 A suitable solution of cellulose, for example in cuprammonia solution, or in a zinc chloride solution, or in a mixture of caustic alkali solution with guanidine or with urea or thiourea or another suitable member of the group of ammonia derivatives of  $\text{CO}_2$  or  $\text{CS}_2$ , or in a solution of a thiocyanate, for example calcium thiocyanate, or a suitable solution of a conversion or oxidation or degradation product of cellulose, or of mercerized cellulose, in short or any of the cellulosic materials proposed for being employed in the industry of solutions of cellulose, or of a 15 suitable cellulose derivative, such as a suitable cellulose ester of lower stage of esterification, or of a suitable cellulose ether, for example ethyl cellulose or methyl cellulose of a low degree of etherification, or of a suitable N-substituted thiourethane of cellulose, for example a phenyl thiourethane of cellulose, or of cellulose xanthate (viscose)—which expression is intended to include xanthates of cellulose or of its conversion—degradation- or oxidation-products, in short of 20 all cellulosic materials that have been proposed as parent materials for the manufacture of cellulose xanthate, (viscose) or of other cellulose derivatives—or of another suitable cellulose derivative containing a CSS-group, for instance of 25 15 a cellulose xantho-fatty acid, or of a product resulting from contacting a cellulose xanthate (or a xanthate of another cellulosic body or another cellulosic compound containing a CSS-group) with a halogen derivative of a di- or poly- 30 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840

or foam. The experience gained hitherto has however taught me that it is very difficult and in many cases even impossible, by purely mechanical means, to transform the solutions or pastes in question into so stiff, voluminous and 5 stable a lather as they yield when substances capable of creating lather such as bodies belonging to the group of saponins, for example saponin-quillajin (quillaja-saponin), githagin (saponin of agrostemma githago) or the like, 10 proteins, degradation products of the latter such as peptones or albumoses, soaps, "solvenol" (sodium salt of benzyl sulphonic acid) in the presence or absence of sodium carbonate, "monopol" oil, Turkey red oil, "monopol" soap (a well known sulphonated castor oil soap) dyestuffs capable of creating lather or the like are used in conjunction with suitable mechanical means.

15 It must be borne in mind that the really lathery condition of the solutions or pastes being not only 20 characteristic of the present invention, but also the sole factor responsible for the new effect of the present invention, that is for the superior voluminosity, specific gravity, softness, feel and the like of the final products of the present invention, a thorough transformation into a lather and a more or less stiff condition of the lather is 25 essential. In consequence, I prefer to perform the transformation of the solutions or pastes into a lather by means of substances capable of creating lather in combination with effective mechanical means which by themselves in no case give 30 results that are to be compared with the results obtained in presence of lather creators. I also prefer to conduct the transformation of the solutions or pastes into lather in such a manner that the lather attains a certain stiffness and retains 35 its lathery condition, stiffness and voluminosity for a longer time.

40 Since in a lather the fluid is only the dispersion medium, the dispersed phase being a gas, a gas must be present when the solution or paste is transformed into lather. I prefer to use for this purpose air, but, if desired, any other gas, such as nitrogen or hydrogen or carbon dioxide may be 45 used.

45 All the details of the practical carrying out of the second phase of the invention, that is the application of the lather to the textile material, for example the mechanical part of the process, 50 or the precipitating baths, or the washing methods, or the bleaching methods or, if derivatives containing the CSS-group are used as parent materials, the desulphurizing methods, or the 55 finishing and drying methods and the like, or the evaporative methods when drying processes are used, belong to the well known and frequently described methods of producing coatings, fillings, or artificial leather, or book cloth or the like from the said cellulosic bodies.

60 It is self-evident that in the course of the treatment of textile materials according to the invention, in all cases in which solutions of cellulose or solutions of such conversion products or derivatives of cellulose are used as are insoluble 65 in water or organic, volatile solvents, the cellulose or the conversion products of cellulose or the cellulose derivatives must be precipitated or regenerated by means of suitable precipitating or coagulating agents, which, if desired, may also 70 exert a plasticising action on the freshly coagulated material.

75 I note that in my U. S. Patent 1,829,904 and in my U. S. application 367,155, filed May 29, 1929 (and in a substitute application 51,171 filed 75

Nov. 22, 1935) I have described the application to textile materials of viscose containing gas in solution or in the form of numerous fine bubbles. The disclosure of said patent may serve as a guide with respect to the details of the cloth-finishing art.

I shall now give several examples of my invention, but it will be understood that the invention is not limited to these details. Consequently, many variations may be made therein without departing from the spirit of the invention. The parts are by weight:—

*Example 1 (a) to (d)*

(a) 18 parts of Marseilles soap dissolved in 720 parts of water are added to 1428 parts of a viscose prepared from 100 parts of cellulose and containing about 6.5 per cent. of precipitable cellulose and 8 per cent. of caustic soda. The mixture is filtered two to three times through cotton, whereupon the solution is whisked or beaten until it is transformed into a dense and stiff lather.

A cotton fabric is in known manner impregnated once or (optionally with intermediate drying) several times in a backfilling or padding machine with the lather thus produced.

In either case this is not merely a surface coating but there is a substantial penetration of the substance of the lather into the fabric, i. e. the fabric is "impregnated."

Then the dressed material, in the wet state or after intermediate drying, is introduced into any precipitating bath known in the viscose art, such as the so-called Mueller-bath, for instance a bath containing per litre 160 grams of sulphuric acid monohydrate and 320 grams of sodium sulphate, or 100 parts of sulphuric acid monohydrate and 160 parts of sodium sulphate, or into a bath composed of 64 parts of water, 10 parts of sulphuric acid, 9 parts of glucose, 12 parts of sodium sulphate, 12 parts of ammonium sulphate and 1 to 3 parts of zinc sulphate, or into sulphuric acid of 10 to 20 per cent. strength, the temperature of the bath being 45 to 50° C. or 4 to 8° C. or room temperature.

Instead of a precipitating bath that has only a coagulating effect on the viscose, a so-called Lilienfeld-bath may be used, that is a bath that has a coagulating effect on the viscose and a plasticising effect on the freshly coagulated viscose, the best and cheapest bath answering this purpose being a bath containing a large proportion, for instance not less than 40 per cent. of sulphuric acid monohydrate in presence or absence of other inorganic substances, such as salts, or of organic substances.

The Lilienfeld-process can also be employed in a two-bath system in which case the impregnated material is first introduced into a bath that has only a coagulating effect on the viscose and then into a bath that has a plasticising effect on the freshly coagulated viscose.

As far as viscose is concerned, all baths known in the viscose art and/or in the art of making artificial materials, particularly threads from any alkali-soluble derivatives or conversion products and from alkaline cellulose solutions are meant to be included in the expression "coagulating baths" or "coagulating agents" wherever this expression is used to define such baths as have little or no plasticising effect on the freshly coagulated material. Consequently, not only the so-called Mueller-bath or any modification thereof come into consideration as coagulating baths in the present process, but all baths

known in the viscose art regardless of whether or not, in addition to the purely coagulating constituents, such as acids and/or acid or neutral salts, they contain any other inorganic or organic (liquid, oily, crystalline or colloidal) substance or substances.

As far as plasticising baths are concerned, particularly suitable are such baths as contain not less than about 30 to 40, preferably not less than 45 per cent. of  $H_2SO_4$ , or an equivalent quantity of another mineral acid. Other agents exerting a similar effect may however be used, for instance, baths consisting of, or containing by itself or in admixture with one or more other organic or one or more inorganic substances, a large proportion of one or more of the following bodies:

Acid esters formed from a polybasic inorganic acid and a monohydric or polyhydric aliphatic or aromatic alcohol (for example methylsulphuric or ethylsulphuric acid or a mixture of methyl or ethyl alcohol or of one of their hydrates with concentrated sulphuric acid), or

Sulphonic acids of aliphatic or aromatic hydrocarbons (for example oxy-(hydroxy)-methylsulphonic acid or methionic acid or methyl- or ethylsulphonic acid or a sulphonic acid of a mineral oil or benzene-sulphonic acid or phenol-sulphonic acid by itself or in admixture with sulphuric acid), or

Carboxy-organo-mineral acids (for example sulphono-di-acetic acid or sulpho-acetic acid by itself or in admixture with sulphuric acid), or

Aromatic sulpho-acids containing nitrogen by themselves or in admixture with sulphuric acid, or

Baths in which sulphuric acid of less than 55 per cent. strength is used in combination with acid salts, such as bisulphates, for instance ammonium bisulphate, or

Strong sulphuric acid containing formaldehyde or pyridine or another organic substance, or

Solutions of zinc halides alone or mixed with an acid or with another salt or both, or

Any other plasticising agent or equivalent for strong mineral acid.

The strong sulphuric acid or other mineral acids or other plasticising agents mentioned above may be used alone or (so far as is in conformity with the conditions of operation) mixed with one or several inorganic substances, for instance with one or several other strong mineral acids, such as hydrochloric acid, nitric acid, or phosphoric acid, or with a neutral or acid salt, such as sodium sulphate or sodium bisulphate, or ammonium bisulphate, ammonium sulphate, magnesium sulphate, zinc sulphate, sodium bisulphite, sodium sulphite, sodium nitrite or boric acid. To the plasticising agents (such as strong sulphuric acid or another mineral acid or the other plasticising agents mentioned above) or to a mixture of these with another strong acid or with one or several of the above-named inorganic substances, may be added (so far as is in conformity with the conditions under which the mineral acids or other plasticising agents are used) a suitable quantity of one or several organic substances, such as glycerine, or a sugar, such as glucose, or an alcohol, or a salt of an organic base, for instance an aniline salt, or pyridine, or a pyridine salt, or an aldehyde, or an organic acid, such as acetic acid, or formic acid, or lactic acid, or oxalic acid.

In the impregnated material, the cellulose may also be regenerated by other methods, for exam-

ple by steaming or heating the material, or by allowing the coated or impregnated textile material to remain at room temperature until the regeneration of the cellulose occurs.

5 The material is washed, dried and finished in the usual manner.

It will be understood that the material may be desulphurised or bleached in any known manner before or after it has been dried.

10 (b) The process is conducted as in (a), but with the difference that only 5 parts of Marseilles' soap are used.

(c) The process is conducted as in (a), but with the difference that 50 to 70 parts of Marseilles' soap are used.

15 (d) The process is conducted as in (a) or (b) or (c), but with the difference that, instead of Marseilles' soap, another soap, for example ordinary shaving soap, or "monopol" soap, or "sol-venol" and sodium carbonate, or "monopol" oil, or Turkey red oil, or a mixture of Turkey red oil and soap, or a peptone, or an albumose, or albumen, or saponin is used.

*Example 2 (a) to (d)*

25 The process is conducted as in any one of the Examples 1 (a) to (d), but with the difference that 100 to 300 per cent. (calculated on the cellulose contained in the viscose) of French chalk or china clay are added to the viscose before or after it has been transformed into lather.

*Example 3 (a) to (d)*

Mode of procedure as in any one of the Examples 1 (a) to (d), but with the difference that the initial viscose contains 8.26 per cent. of precipitable cellulose and 9.4 per cent. of caustic soda solution and that the substance creating lather is dissolved in 300 parts of water. The volume of the final lather is about three times 35 as large as the volume of the viscose before it has been transformed into the lather.

*Example 4 (a) to (d)*

45 Mode of procedure as in any one of the Examples 3 (a) to (d), but with the difference that, instead of 18 parts, 5 parts of Marseilles' soap are used. The volume of the final lather is about three and a half times as large as the volume of the viscose before it has been transformed into the lather.

*Example 5 (a) to (d)*

The process is conducted as in any one of the Examples 3 (a) to (d), but with the difference that the initial viscose contains 8.26 per cent. of cellulose and 5.9 per cent. of caustic soda.

*Example 6 (a) to (d)*

Mode of procedure as in any one of the Examples 3 (a) to (d), but with the difference that the initial viscose contains 8.26 per cent. of cellulose and 3.8 per cent. of caustic soda.

*Example 7 (a) to (d)*

65 The process is conducted as in any one of the Examples 1 (a) to (d), but with the difference that the viscose is prepared from a very viscous cellulose rich in alpha-cellulose (for instance from very viscous cotton linters or the so-called 70 alpha-fibre cellulose), and that the substance creating lather is dissolved in 1905 parts of caustic soda solution of 2.7 per cent. strength.

*Example 8 (a) to (d)*

75 Mode of procedure as in any one of the Ex-

amples 7 (a) to (d), but with the difference that the initial viscose contains 7 per cent. of precipitable cellulose and 11.3 per cent. of caustic soda solution and that 5 parts of Marseilles' soap dissolved in 1905 parts of water are added. 5

*Example 9 (a) to (d)*

The process is conducted as in any one of the Examples 1 (a) to (d), but with the difference that the initial viscose contains about 14 10 per cent. of cellulose and about 10 per cent. of caustic soda (to have a manageable degree of viscosity in spite of its high content in cellulose, the viscose is prepared from an alkali cellulose that has been allowed to mature for a long time, say 96 to 120 hours), and that the substance creating lather is dissolved either in 714 parts of water or in 714 parts of caustic soda solution of 3 per cent. strength.

*Example 10 (a) to (d)*

Mode of procedure as in any one of the Examples 1 (a) to (d), but with the difference that the initial viscose contains 8 per cent. of cellulose and 12 per cent. of caustic soda, and that the substance creating lather is dissolved in 750 parts of water.

*Example 11*

An alkali cellulose containing about 100 parts 39 of parent cellulose, 36 parts of caustic soda and 264 parts of water is treated with carbon bisulphide in the usual manner and the thus obtained product is dissolved in a solution of 5 to 10 per cent. of one of the substances creating lather set forth in Example 1, in 1068 parts of water, or in 1068 parts of a caustic soda solution of 2.8 per cent. strength, or in 1068 parts of caustic soda solution of 6.5 per cent. strength or in 2973 parts of caustic soda solution of 4.2 40 per cent. strength.

The lather thus obtained is employed for impregnating cloth according to Example 1.

*Example 12*

400 to 600 parts of caustic soda solution of 20 per cent. strength are added in small portions to 100 parts of cellulose placed in a shredder or a vacuum xanthate machine of Werner and Pfleiderer and the mass kneaded or shredded respectively until homogeneous, whereupon 60 parts of carbon bisulphide are added and the kneading is continued for another 2 to 3 hours.

After that time, the excess carbon bisulphide is blown off and 5 to 50 parts of one of the substances creating lather set forth in Example 1 and dissolved in 668 parts of water, or in 868 parts of water, or in 1240 parts of water, or in 1440 parts of water, or in 1740 parts of water, or in 1940 parts of caustic soda solution of 2.3 per cent. strength, are added to the viscose whereupon the mixture thus obtained is brought into a lathery condition as described in Example 1 and then used for impregnating a cotton fabric according to the prescription given in Example 1.

*Example 13*

The process is conducted as in any one of the preceding examples, but with the difference that, instead of viscose, a solution of a phenyl thiourethane of cellulose (for example prepared according to the process described in my Patent No. 1,674,401) dissolved in a proportion of water and caustic soda corresponding with the proportions contained in the viscoses employed.

in the foregoing examples is used as initial material.

*Example 14*

5 The process is conducted as in any one of the preceding examples, but with the difference, that, instead of being introduced into a coagulating or coagulating and plasticising bath, the impregnated material is dried and thereafter steamed for 3 to 10 minutes and then washed and dried. After being washed, the material may be taken through a dilute acid, then washed again and dried.

*Example 15*

15 The process is conducted as in any one of the foregoing examples, but with the difference that the impregnated material is, at any stage of manufacture subsequent to the coagulating step, introduced into a solution of a shrinking agent, for example into a caustic soda solution of 7 per cent. strength, or into a caustic soda solution of 22 per cent. strength and then washed and dried.

Instead of viscose, a solution of cellulose or of a conversion product of cellulose in cuprammonia or caustic soda solution containing thiourea or guanidine (see my U. S. patent No. 1,771,460 and No. 1,771,461), or in calcium thiocyanate can be used in the present invention.

Also solutions or pastes of cellulose esters, such as cellulose acetate or cellulose nitrate or of cellulose ethers, such as ethyl or methyl ether of cellulose of low degree of etherification can be brought into a lather condition by means of the described methods and the lather employed as a coating.

*Example 16*

The process is conducted as in any one of the Examples 1 to 15, but with the difference that 10 to 30 parts (calculated on the cellulose contained in the viscose) of  $\alpha$ -dichlorohydine, or monochlorohydine, or ethylene chlorohydine, or 20 to 50 parts of one of the products described, or mentioned in my U. S. Patent 2,100,968 or used 40 in my U. S. application Ser. No. 597,640 respectively, or 20 parts of  $\alpha$ -dichlorohydine and 20 parts of one of the products described or mentioned in my U. S. Patent 2,100,968 or used in my co-pending U. S. application Ser. No. 597,640 respectively, or 20 parts of  $\alpha$ -dichlorohydine and 20 to 50 parts of one of the products described or mentioned in my British Patents 390,516 or 390,523 or used in my U. S. Patent 2,051,051 respectively, or 20 to 30 parts of one or more reagents belonging to the group set forth in my U. S. Patent 2,021,864 are added to the viscose.

The expression "cellulose" is, wherever the context permits, intended to denote not only cellulose, but also its conversion products, for example its hydrates or degradation products or oxidation products.

It is to be understood that in the following claims the term "applying to textile material" includes any manner of application to the textile material, whether by manual or mechanical means customary for dressing, sizing, filling, impregnating, coating, weighting or printing textile material, whether in the state of woven fabrics, or in the state of yarn.

70 The term "lather" as used in the specification and claims is not to be limited to a foam or froth produced only by reason of the presence of soap or its equivalent.

The expression "textile material" in the specification and the claims includes, wherever the

context permits, any spun or woven textile material, whether animal or vegetable (for example, flax, linen, hemp, ramie, jute, wool, and particularly cotton) as well as artificial fibres of any kind in the form of yarn, staple fibre or fabrics consisting of, or containing artificial fibres, in the form of pure fabrics, or in the form of mixed fabrics, or in the form of yarn in skeins, cops or warps.

The invention embraces the production of 10 coatings, impregnations and layers of every kind; dressings upon textiles, paper, leather and the like; sizing upon yarns; book cloth; artificial leather; plates, etc., whether or not they also include fillers, coloring agents and the like. 15

In the claims, the term "solution of cellulosic material" is intended to cover freely liquid solutions, solutions of high viscosity, pastes and the like, as hereinabove described. The term "insoluble cellulosic material" is intended to cover regenerated cellulose, and regenerated cellulose derivatives or compounds, including those produced by coagulating and/or plasticizing from the solutions or pastes described above. The term "solution of a xanthate of a cellulosic compound" is 20 intended to cover viscose and the products made by contacting viscose with an organic substance, of the kinds mentioned herein, capable of acting on the viscose without coagulating the latter. This term includes solutions of xanthates of cellulose and of cellulose derivatives. 25

The expression "strong mineral acids" denotes sulphuric acid of at least 30 per cent. of  $H_2SO_4$ , preferably at least 45 per cent. of  $H_2SO_4$ , and as regards the other mineral acids, solution of 30 equivalent strength.

The expression "strong sulphuric acid" or "sulphuric acid containing at least about 30 per cent. of sulphuric acid monohydrate" denotes sulphuric acid having a content of 30 to 98 per cent. of  $H_2SO_4$ . 35

What I claim is:

1. A treatment of textile material which comprises converting a solution containing a dissolved cellulosic material into a lather, and applying said lather to a textile material. 45

2. A treatment of textile material which comprises applying thereto a lather of a solution of a cellulosic material and treating the material so as to convert the soluble cellulosic material into 50 an insoluble cellulosic material while bonded to said textile material.

3. A treatment of textile material, which comprises transforming a solution of a cellulosic material into a lather, applying the lather to the 55 textile material, and regenerating an insoluble cellulosic material from said solution in a highly porous state.

4. A treatment as claimed in claim 1 wherein the original cellulosic solution is a solution containing a cellulose derivative. 60

5. A process as claimed in claim 1, wherein the solution to be transformed into lather, is a solution of an alkali-soluble cellulosic material.

6. A process as claimed in claim 1, wherein the solution of the compound of cellulose is viscose. 65

7. A process as claimed in claim 1, wherein the compound of cellulose is a xanthate of a cellulose derivative. 70

8. A treatment as claimed in claim 1, wherein the transformation of the solution containing a soluble cellulosic material, into a lather is effected with the aid of suitable mechanical means. 75

9. A treatment as claimed in claim 1, wherein the transformation of the solution into lather is effected with the aid of at least one substance having lather forming properties.
- 5 10. A treatment as claimed in claim 1, wherein in the transformation of the solution into lather is effected with the aid of at least one substance having lather-forming properties, in combination with suitable mechanical means.
- 10 11. A treatment as claimed in claim 1, wherein soap is present to assist the formation of the lather.
- 15 12. A treatment as claimed in claim 1, wherein the solution is transformed into a lather, in the presence of a body belonging to the group of saponins.
- 20 13. A treatment of textile material which comprises applying to the textile material a lather produced of a solution of an alkali-soluble cellulosic material and then treating the material with an agent having a coagulating effect on the lather applied to the textile material and a plasticizing effect on the freshly coagulated lather.
- 25 14. A treatment of textile material which comprises applying to the textile material, a lather produced of a solution containing a dissolved alkali-soluble cellulosic material and then treating the material first with an agent which has a coagulating effect on the lather applied to the textile fibre and then with an agent which has a plasticizing effect on the freshly coagulated cellulosic material from said lather.
- 30 15. A process which comprises treating a lather while intimately associated with a textile fabric, which lather contains a solution containing a dissolved cellulosic material, with an acid solution which is capable of regenerating an insoluble cellulosic material from said solution.
16. A process which comprises treating a lather in a preshaped state, which lather contains a solution of a cellulosic material, with an acid solution which is capable of regenerating an insoluble cellulosic material from said solution. 5
17. Textile material, carrying intimately bonded thereto, an insoluble cellulosic material which has been produced by impregnating a textile material with a lather containing a dissolved cellulosic material and regenerating an insoluble cellulosic material from said dissolved cellulosic material, said product having a warm feel 10 and being of a downy character.
18. A process of dressing or sizing a textile material which comprises applying a lather containing as a constituent, a dissolved cellulosic 20 body, to said textile material, forcing the substance of the lather into the body of the textile material to impregnate the same, and thereafter treating the so impregnated textile material with an agency capable of coagulating a 25 cellulosic substance in said textile material.
19. The herein described process of sizing textile material which comprises converting a solution containing a dissolved cellulosic body into the state of a lather, impregnating a textile 30 material therewith, and converting the dissolved cellulosic body into an undissolved cellulosic body which is insoluble in water.

LEON LILIENFELD.